

# UNITED STATES PATENT OFFICE.

SAMUEL GROSSIORD, OF LES MOUSSIÈRES, FRANCE.

## METHOD OF PRODUCING ARTIFICIAL PRECIOUS STONES.

SPECIFICATION forming part of Letters Patent No. 297,598, dated April 29, 1884.

Application filed December 17, 1883. (No specimens.) Patented in France October 25, 1883, No. 151,732.

*To all whom it may concern:*

Be it known that I, SAMUEL GROSSIORD, a citizen of the French Republic, residing at Les Moussières, in the Republic of France, have invented certain Improvements in the 5 Method of Producing Artificial Precious Stones, (for which I have obtained Letters Patent in France, under date of October 25, 1883, No. 151,732;) and I do hereby declare the 10 following to be a full, clear, and exact description of the same.

My present invention relates to improvements in the art of producing artificial precious stones as described in Letters Patent of the 15 United States granted to me under date of July 3, 1883, No. 280,467, and under date of December 11, 1883, No. 290,040.

The object of this invention is to produce, with facility and at little expense, multi-colored 20 artificial precious stones, or artificial stones of a given color, by the association of enamels of different colors with or without strass. These artificial precious stones I have denominated "colored or multi-colored diamondines."

25 The present invention may be carried into practical effect in various ways, which necessarily depend on the nature of the gem to be produced, its color, and brilliancy.

In general, for producing a gem of uniform 30 color, or of a variegated color, of medium brilliancy, I take a suitable receiver or crucible having a series of cells or holes, either cylindrical, square, octagonal, or of other form in cross-section, and of a capacity equal to, or 35 nearly equal to, the size of stone to be obtained, said cells having a flat bottom. In these cells I place, in superposed layers, first a piece of strass and on top of this alternate layers of enamel of different colors, to produce either a 40 gem of a given color, or one of different colors, or variegated. These are then subjected to heat, and either fritted, fused, or melted together. According to the brilliancy and the depth of color the stone is to have, the above

method will be varied—as, for instance, a piece 45 of strass may be interposed between any two or more pieces of enamel and the whole fritted, fused, or melted together; nor is it necessary that the enamel employed should be previously polished. If desired, instead of producing 50 each stone separately, a block or large stone may be produced from which the stones may be cut and then prepared for setting. The strass may also be dispensed with and a multi-colored stone obtained, or a stone of a given 55 color, by the combined colors of the enamel.

Having described my invention, what I claim is—

1. The herein-described method of obtaining artificial precious stones, which consists 60 in fritting, fusing, or melting together superposed layers of colored enamels, as described.

2. The herein-described method of obtaining imitation precious stones of a given color or of a variegated color, which consists in 65 fritting, fusing, or melting together superposed layers of colored enamels to a foundation-layer of strass, as described.

3. The herein-described method of obtaining imitation precious stones of a given color, 70 or of variegated colors, which consists in fritting, fusing, or melting together alternating superposed layers of strass and colored enamels, as described.

4. As a new article of manufacture, an 75 imitation precious stone composed of enamels of different colors, as set forth.

5. As a new article of manufacture, an imitation precious stone composed of enamels of different colors and strass, as described. 80

In testimony that I claim the foregoing I have hereunto set my hand this 18th day of October, 1883.

SAM. GROSSIORD.

Witnesses:

CAMILLE CHARROPPIN,  
EMILE KANTER.